

1

2,747,991

## MAGNESIUM-BASE ALLOYS

Alfred H. Hesse, Worthington, Ohio, assignor, by mesne assignments, to Olin Mathieson Chemical Corporation, a corporation of Virginia

No Drawing. Application September 14, 1945,  
Serial No. 616,161

1 Claim. (Cl. 75—168)

This invention relates to magnesium-base alloys and has for its object the provision of an improved magnesium-base alloy comprising lithium as an essential constituent, together with one or more other alloying metals. More particularly, the invention provides an alloy comprising magnesium as the principal constituent, from around 1% to 13% of lithium, and one or more other metals, as described hereinafter, which modify and improve the physical characteristics of the basic alloy of magnesium and lithium.

Alloys of the invention are characterized by low specific gravity, good ductility, high tensile strength and good working properties. A number of these alloys have good creep resistance and stability of tensile strength at room temperature and some are susceptible of heat treatment.

In accordance with my invention, I provide various alloys of magnesium and lithium together with other beneficial metals to form ternary, quaternary and quinary alloys having important physical characteristics. As beneficial metals in the magnesium and lithium basic structure which I have found and confirmed as useful are the following: Aluminum, antimony, barium, beryllium, bismuth, cadmium, cerium, calcium, chromium, copper, indium, lead, manganese, molybdenum, nickel,

2

silicon, silver, strontium, tantalum, thallium, tin, titanium, vanadium, and zinc.

The new alloys of the invention may be prepared by any of the usual melting processes with precautions to prevent an excessive sodium contamination. For example, the magnesium may be melted in an iron crucible under a suitable flux, and then the beneficial metal or metals are added, followed by the addition of lithium. In order to avoid excessive oxidation of the lithium during the alloying process, it is advisable to use means for holding the lightweight lithium beneath the surface of the molten metal. An inverted perforated steel cup, such as a phosphorizing cup or an analogous device suitable for this purpose, may be used. Temperatures of about 1300° to 1400° F. may be used for alloying operations. After thorough agitation to insure homogeneity, the melt is allowed to settle at temperatures sufficient to maintain it in a liquid state, after which it is decanted into molds. A suitable casting temperature is, for example, about 1320° F. The alloy may be cast directly into permanent molds without the necessity of providing a neutral or reducing atmosphere.

To insure the absence of harmful amounts of sodium or potassium, I prefer to prepare these alloys as described in my copending application, Serial No. 603,749, filed July 7, 1945, now Patent No. 2,507,713, issued May 16, 1950. In accordance with that application, I may use a flux made up of one part of lithium fluoride to three parts of lithium chloride. Use of such a flux serves to reduce the sodium and potassium content of the alloy. I may also treat the alloy by blowing the melt with a gas, such as nitrogen or ammonia, to accomplish a decrease in sodium or potassium.

As an illustration of the lightness of these alloys, most of them are lighter than magnesium, having specific gravities around 1.55.

Illustrative examples of alloys of this invention and certain of their physical properties are given in the following table:

| No.     | Percentages |       |      |    |    | Per Cent Elongation | Per Cent Reduction in Area | Yield Strength | Tensile Strength |
|---------|-------------|-------|------|----|----|---------------------|----------------------------|----------------|------------------|
|         | Mg          | Li    | Sn   | Pb | Cd |                     |                            |                |                  |
| 1.....  | 94.08       | 3.92  | 2    |    |    | 9.5                 | 20.8                       | 24,500         | 33,200           |
| 2.....  | 79.70       | 8.30  | 12   |    |    | 9.3                 | 10.8                       | 19,000         | 25,300           |
| 3.....  | 95.04       | 3.96  | 1    | Pb |    | 13.5                | 27.3                       | 18,900         | 28,100           |
| 4.....  | 79.70       | 8.30  | 12   |    | Cd | 34.3                | 38.9                       | 19,300         | 25,200           |
| 5.....  | 94.08       | 3.92  | 2    |    |    | 20.7                | 42.6                       | 15,800         | 25,400           |
| 6.....  | 92.16       | 3.84  | 4    |    | Bi | 18.7                | 41.4                       | 16,100         | 26,900           |
| 7.....  | 94.08       | 3.92  | 2    |    |    | 16.0                | 33.7                       | 16,300         | 24,700           |
| 8.....  | 85.17       | 8.83  | 6    |    | Cu | 36.0                | 60.3                       | 15,500         | 21,100           |
| 9.....  | 88.10       | 10.90 | 1    |    |    | 42.0                | 74.5                       | 18,700         | 21,700           |
| 10..... | 92.16       | 3.84  | 4    |    | Mn | 16.0                | 30.6                       | 15,900         | 28,300           |
| 11..... | 87.22       | 10.78 | 2    |    |    | 38.0                | 73.9                       | 13,900         | 18,000           |
| 12..... | 92.16       | 3.84  | 4    |    | Ca | 9.9                 | 19.5                       | 20,400         | 28,700           |
| 13..... | 90.17       | 8.5   | 1.08 |    | Sr | 16.2                | 27.0                       | 23,800         | 29,700           |
| 14..... | 94.08       | 3.92  | 2    |    |    | 21.2                | 40.3                       | 14,900         | 24,700           |
| 15..... | 87.0        | 9.0   | 4    |    |    | 43.0                | 60.5                       | 16,200         | 21,000           |
| 16..... | 95.04       | 3.96  | 1    |    | Ag | 20.0                | 45.5                       | 17,500         | 27,200           |
| 17..... | 87.0        | 9.0   | 4    |    | Ni | 43.7                | 68.8                       | 21,100         | 26,800           |
| 18..... | 95.04       | 3.96  | 1    |    |    | 17.0                | 37.5                       | 17,200         | 27,800           |
| 19..... | 81.88       | 10.12 | 8    |    |    | 44.2                | 50.9                       | 17,900         | 23,900           |
| 20..... | 95.04       | 3.96  | 1    |    | Sb | 17.7                | 39.8                       | 16,000         | 25,100           |
| 21..... | 87.0        | 9.0   | 4    |    |    | 44.0                | 59.4                       | 16,600         | 21,500           |
| 22..... | 95.04       | 3.96  | 1    |    |    | 16.7                | 21.6                       | 19,200         | 25,700           |
| 23..... | 87.0        | 9.0   | 4    |    |    | 16.2                | 16.4                       | 18,900         | 24,700           |
| 24..... | 85.26       | 8.82  | 3.92 | 2  | Al | 28.2                | 49.2                       | 29,800         | 35,900           |

| No. | Percentages |         |         |            |  | Per Cent Elonga-tion | Per Cent Reduc-tion in Area | Yield Strength | Tensile Strength |
|-----|-------------|---------|---------|------------|--|----------------------|-----------------------------|----------------|------------------|
| 25  | Mg 84.64    | Li 7.36 | Sn 4.00 | In 4       |  | 17.7                 | 23.9                        | 31,600         | 41,500           |
| 26  | 95.04       | 3.96    | 1       |            |  | 19.0                 | 35.9                        | 15,800         | 24,900           |
| 27  | 95.04       | 3.96    | 1       | Be         |  | 19.0                 | 42.0                        | 16,400         | 26,200           |
| 28  | 93.12       | 3.88    | 2.7     | Ce         |  | 13.5                 | 20.4                        | 20,300         | 28,100           |
| 29  | 89.74       | 8.87    | 1.39    | Ba         |  | 35.7                 | 54.0                        | 18,300         | 24,200           |
| 30  | 85.26       | 8.82    | 3.92    | Zn Mn 2    |  | 39.5                 | 65.7                        | 24,600         | 31,200           |
| 31  | 81.88       | 10.12   | 8       | Cu         |  | 41.7                 | 44.1                        | 18,300         | 24,000           |
| 32  | 83.37       | 8.63    | 8       | Ni         |  | 35.7                 | 39.7                        | 19,900         | 27,300           |
| 33  | 89.74       | 9.26    | 1       | In         |  | 46.2                 | 64.9                        | 20,800         | 24,500           |
| 34  | 89.74       | 9.26    | 1       | Be         |  | 44.0                 | 67.1                        | 16,100         | 21,000           |
| 35  | 87.9        | 9.1     | 3       | Mn         |  | 43.2                 | 50.9                        | 16,900         | 22,800           |
| 36  | 90.0        | 10.0    | .007    | Cr         |  | 42.2                 | 72.1                        | 14,100         | 19,100           |
| 37  | 86.08       | 8.92    | 4       | Zn Ni 1    |  | 35.0                 | 62.0                        | 24,100         | 29,700           |
| 38  | 88.8        | 8.8     | 0.76    | Sr         |  | 46.2                 | 64.9                        | 12,900         | 21,800           |
| 39  | 91.0        | 9.1     | 1.18    | Ba         |  | 35.7                 | 54.0                        | 18,300         | 24,200           |
| 40  | 89.7        | 9.3     | 1       | Sn         |  | 41.5                 | 62.8                        | 17,500         | 20,900           |
| 41  | 86.1        | 8.9     | 4       | Zn Cu 1    |  | 34.7                 | 62.8                        | 22,600         | 28,600           |
| 42  | 81.9        | 10.1    | 4       | Zn Ni 4    |  | 28.0                 | 46.8                        | 22,300         | 29,400           |
| 43  | 81.9        | 10.1    | 4       | Zn Si      |  | 10.5                 | 14.8                        | 24,100         | 31,700           |
| 44  | 84.6        | 10.4    | 4       | Cu         |  | 36.5                 | 68.0                        | 21,200         | 27,100           |
| 45  | 87.4        | 3.6     | 8       | Al Cu 1    |  | 7.5                  | 9.6                         | 31,900         | 44,400           |
| 46  | 88.8        | 9.2     | 1       | Al Ni      |  | 29.7                 | 65.5                        | 23,200         | 27,400           |
| 47  | 84.3        | 8.7     | 6       | Al Be      |  | 7.7                  | 9.4                         | 32,000         | 39,500           |
| 48  | 84.3        | 8.7     | 6       | Al Cu      |  | 13.7                 | 14.3                        | 31,400         | 39,200           |
| 49  | 84.3        | 8.7     | 6       | Al Mn      |  | 9.7                  | 12.1                        | 31,600         | 38,800           |
| 50  | 83.4        | 8.6     | 6       | Al Sr      |  | 12.0                 | 17.2                        | 31,900         | 38,300           |
| 51  | 87.2        | 10.8    | 1       | Cu         |  | 27.2                 | 54.7                        | 26,500         | 29,300           |
| 52  | 84.5        | 10.5    | 1       | Al Ni      |  | 39.0                 | 68.8                        | 18,000         | 22,800           |
| 53  | 84.5        | 10.5    | 1       | Al Si      |  | 6.2                  | 10.6                        | 29,500         | 33,700           |
| 54  | 90.2        | 3.8     | 2       | Sn Ag      |  | 16.0                 | 41.2                        | 25,000         | 37,300           |
| 55  | 90.2        | 3.8     | 2       | Sn Zn      |  | 16.5                 | 36.5                        | 26,500         | 39,800           |
| 56  | 88.3        | 3.7     | 2       | Zn Al Sn 2 |  | 13.7                 | 14.6                        | 33,300         | 47,400           |
| 57  | 87.0        | 9.0     | 2       | Zn Al Mn   |  | 25.0                 | 56.8                        | 31,200         | 35,500           |
| 58  | 87.0        | 9.0     | 2       | Zn Al Cu   |  | 27.0                 | 58.8                        | 29,400         | 33,700           |
| 59  | 87.0        | 9.0     | 2       | Zn Al Ni   |  | 30.2                 | 60.4                        | 28,900         | 32,600           |
| 60  | 85.4        | 10.6    | 2       | Zn Al Cu   |  | 25.2                 | 56.6                        | 28,900         | 32,500           |
| 61  | 82.8        | 10.2    | 2       | Zn Al Ni   |  | 36.2                 | 65.6                        | 20,800         | 25,700           |
| 62  | 82.8        | 10.2    | 2       | Zn Al Si   |  | 5.2                  | 9.5                         | 31,100         | 35,100           |
| 63  | 84.6        | 6.4     | 4       | Zn Cd Al   |  | 27.0                 | 38.5                        | 24,100         | 34,800           |
| 64  | 84.6        | 10.4    | 4       | Cd Al      |  | 26.0                 | 56.0                        | 31,800         | 33,700           |
| 65  | 84.6        | 10.4    | 4       | Cd Cu      |  | 38.7                 | 55.1                        | 19,700         | 25,000           |
| 66  | 83.7        | 10.3    | 2       | Al Ag      |  | 29.2                 | 52.6                        | 28,000         | 32,900           |
| 67  | 81.9        | 10.1    | 4       | Al Cu      |  | 21.7                 | 36.0                        | 31,800         | 36,900           |
| 68  | 84.5        | 10.5    | 1       | Al         |  | 37.8                 | 61.5                        | 16,000         | 22,300           |

I claim:

A magnesium-base alloy consisting of about 2% of zinc, about 4% of aluminum, about 2% of tin, about 3.7% of lithium, with the balance being magnesium.

65

524,113  
361,086  
509,024

## FOREIGN PATENTS

Great Britain ----- July 30, 1940  
Germany ----- Oct. 10, 1922  
Germany ----- Oct. 6, 1930

## References Cited in the file of this patent

70

## UNITED STATES PATENTS

2,226,550 Burkhardt ----- Dec. 31, 1940  
2,261,905 Nelson et al ----- Nov. 4, 1941  
2,305,825 Burkhardt ----- Dec. 22, 1942  
2,317,980 Dean ----- May 4, 1943 75

Serial No. 303,611, Burkhardt (A. P. C.), published May 4, 1943.  
Henry et al., "Lithium-Magnesium Equilibrium Diagram," Trans. Amer. Inst. Mining and Metallurgical Engrs., 1934, vol. III, pp. 319-332.

## OTHER REFERENCES